

## UNITED STATES PATENT OFFICE

2,436,059

## DISCHARGE PRINTING OF COLORED CELLULOSE ACETATE FABRICS WITH THE AID OF AN INTERMEDIATE THIOLCYANATE TREATMENT

Herbert G. Scull and James G. McNally, Rochester, N. Y., assignors to Eastman Kodak Company, Rochester, N. Y., a corporation of New Jersey

No Drawing. Application March 4, 1943,  
Serial No. 478,005

8 Claims. (CL 8—64)

1

This invention or discovery relates to the discharge printing of colored textile fabrics made of or containing an organic derivative of cellulose yarn. More particularly, our invention or discovery is directed to the discharge printing of colored textile fabrics made from an organic derivative of cellulose yarn or yarns or made from an organic derivative of cellulose yarn or yarns in admixture with yarn from materials such as viscose, cotton, cuprammonium silk and regenerated cellulose. Our invention or discovery is particularly directed to the discharge printing of colored textile fabrics made of or containing cellulose acetate.

It is an object of our invention or discovery to provide a process for improving the sharpness of detail and the clearness of the discharged area of colored organic derivative of cellulose textile fabrics subjected to discharge printing operations. A particular object of our invention or discovery is to provide a satisfactory commercial process for the production of white and color discharges in the same pattern on colored textile fabrics containing an organic derivative of cellulose yarn. Another object is to provide a process for producing white and color discharges on colored organic derivative of cellulose textile fabrics by the use of an acid reducing discharge printing paste and an alkaline vat dye color paste. Other objects will appear hereinafter.

Typical organic derivatives of cellulose include the hydrolyzed as well as the unhydrolyzed cellulose organic acid esters such as cellulose acetate, cellulose formate, cellulose propionate or cellulose butyrate and the hydrolyzed as well as the unhydrolyzed mixed organic acid esters of cellulose such as cellulose acetate-propionate, cellulose acetate-butyrate and the cellulose ethers such as methyl cellulose, ethyl cellulose or benzyl cellulose.

Discharge printing processes can be classified under two types known as "discharged dyed style" and "color on color discharge printing." In the first mentioned type the textile fabric is colored with a coloring matter capable of being discharged and a discharge paste is applied in the areas where it is desired to decolorize the colored material. By appropriate treatment the areas where the discharge paste has been applied are left either white or a lighter shade than the original coloring or dyeing while the areas where no discharge paste has been applied are left unchanged.

"Color on color discharge printing" is gener-

2

ally similar to the discharge style described above except that the discharge paste used to destroy the color of the colored fabric contains a dye which colors the area of the fabric which is discharged by the discharge print paste. The dye used in the discharging paste, of course, must not be unduly affected by the discharge paste. In both types of discharge printing the color or dye with which the textile fabric is colored must be one capable of being discharged. The discharge paste, by like token, must be one which is capable of destroying the color of the textile fabric when appropriately applied thereto.

Generally speaking, the discharging of colored textile fabrics is effected through the use of reducing agents. As is well known to those skilled in the art of textile printing, the reduction discharge process based on sodium formaldehyde-sulfoxylate or potassium formaldehyde-sulfoxylate, in general use for the discharging of colored cotton, viscose rayon, cuprammonium silk, silk and wool textile fabrics, has not proven satisfactory for producing clear-cut designs on colored organic derivative of cellulose textile fabrics, such as cellulose acetate. With certain coloring matters, regardless of the concentration of dye used on the ground shade, the discharged areas have a tendency to bleed out or halo around the edges of the printed design. This is more noticeable when the fabric is aged in sufficient moist steam to give good results with vat colors employed in the multi-color patterns as illumination colors, where both white and colored objects are desired in the same pattern.

It has been proposed heretofore to overcome the above-mentioned difficulty of spreading or haloing of the discharge areas and to increase the clearness and sharpness of the discharged areas by incorporating in the discharge paste various acids and swelling agents of an acid nature. These methods have met with some success when the "discharged dyed style" of printing has been carried out and also where a "loose style" of "color on color discharge" has been employed. By a "loose style" is meant a type of printing known to those skilled in the art as the use of colors which are fugitive to light or washing and which are, therefore, limited in their application.

In an effort to secure satisfactory discharges on colored cellulose acetate textile fabrics, the use of calcium thiocyanate or barium thiocyanate (U. S. Patent 1,651,639), zinc thiocyanate (U. S. Patent 1,981,907) or guanidine thiocyanate (U. S. Patent 1,931,108) in the discharge paste, to

produce pastes of an acid character, have been proposed. These pastes apparently give the best results of the prior art discharge printing pastes. However, in producing fast colors with dyes, such as the vat dye colors, which require an alkaline medium, on colored textile fabrics which are to have a pattern containing both white and colored discharges, it has been found that a carry-over from the above-mentioned acid thiocyanate discharge printing pastes gets on the printing roller applying the vat dye color in an alkaline medium. When the carry-over from the acid print paste comes in contact with the alkaline vat dye color, a scum forms on the printing roller applying the vat color. This scum, which is apparently due to the formation of carbonates and oxides by interaction between the acid discharge paste and the alkaline vat dye color, causes smearing of the pattern because the doctor blade is unable to clean properly. Because smearing occurs after the printing operation in question has been in operation but a relatively short time, this method has not proved commercially practical.

While our improved discharge printing process is applicable generally to the discharge printing of colored textile fabrics made of or containing an organic derivative of cellulose yarn, it is of greatest utility for the production of both white and colored discharges on such colored textile fabrics wherein the discharging is effected under acid conditions on a roller printing machine. The textile fabrics, for example, can be prepared from one or more organic derivative of cellulose yarns, or they can be prepared from one or more organic derivative of cellulose yarns in admixture with viscose, cotton or cuprammonium silk yarns, for example.

We have discovered that the objects of our invention or discovery can be accomplished by incorporating an inorganic thiocyanate into the textile fabric prior to the printing operation. Ordinarily the inorganic thiocyanate will be incorporated in the textile fabric after the fabric has been colored but prior to the printing operation. The manner of incorporating the inorganic thiocyanate or the time of its incorporation are immaterial so long as the inorganic thiocyanate is present in the colored textile fabric prior to the printing operation. Thus, the inorganic thiocyanate may be incorporated in the textile fabric by immersion, padding, or spraying, for example. That is, the colored textile fabric may be immersed in a solution of the inorganic thiocyanate, padded with the solution or sprayed with the solution. The colored textile fabric containing the inorganic thiocyanate is dried or substantially dried prior to the printing operation.

Inorganic thiocyanates that can be employed include, for example, calcium thiocyanate, zinc thiocyanate, aluminum thiocyanate, manganous thiocyanate, magnesium thiocyanate, barium thiocyanate, sodium thiocyanate and potassium thiocyanate. For purposes of clarity it is here noted that the thiocyanates are also known as sulfocyanides. Thus, calcium thiocyanate and calcium sulfocyanide are one and the same compound. The use of an acid thiocyanate, such as the first six thiocyanates named above, is generally advantageous.

As previously indicated, the advantages of our invention or discovery are greatest when both white and colored discharges on the colored dyed textile fabric are desired and the discharging is

effected under acid conditions. However, we have found that material advantages are obtained by incorporating an inorganic thiocyanate into the dyed textile fabric prior to printing, rather than applying the thiocyanate through the medium of a printing paste alone. Specifically, the clearness of the discharged area as well as the sharpness of the discharged area is ordinarily improved—two very important advantages. Again, in the case of screen printing, our invention or discovery possesses the added advantage that considerably more pieces of goods (roughly, 2 to 3 times more) may be printed before the screen is rendered unsuitable for use. This advantage is obtained because the thiocyanate in the usual printing pastes attacks the screen, which is ordinarily made from pure silk, nylon or vinyl acetate-vinyl chloride copolymers, whereas if the thiocyanate is incorporated in the colored textile fabric it has little or no effect on the screen. The use of an acid inorganic thiocyanate is preferred by us because we have found that the results obtained using the acid inorganic thiocyanates are, generally speaking, superior to the results obtained when a neutral thiocyanate such as sodium thiocyanate or potassium thiocyanate is used.

Advantageously, when a colored organic derivative of cellulose textile fabric is treated in accordance with our invention or discovery the inorganic thiocyanate is incorporated into the colored textile fabric in conjunction with an appropriate swelling agent. The use of a suitable swelling agent aids in securing good discharge of the color from colored organic derivative of cellulose textile fabrics. Suitable swelling agents, include, for example, organic polyhydric alcohols such as glycerol, diethylene glycol, triethylene glycol, propylene glycol, tetraethylene glycol and thiodiglycol. The high-boiling water-soluble organic swelling agents named are indicated to be illustrative and not limitative as other substances which effect swelling, such as



mono-N-n-butyrylethanolamine



and disalicylethanolamine



and which do not enter into chemical reaction with the printing pastes or the inorganic thiocyanates can be employed. Thiodiglycol, triethylene glycol and



in the order named appear to be best swelling agents for cellulose acetate.

The amounts of the inorganic thiocyanate which should be incorporated into the colored textile fabric vary so widely that definite limits cannot be given. The amount to be used depends, for example, upon the nature of the fabric, the weave of the cloth, the size of the filaments, the dyestuff employed, the depth of the dyeing, the speed of the printing machine, the depth of the engraving and the amount of padding liquor left in the fabric after padding and before drying. For the foregoing reasons it will be apparent that definite limits on the amount of the inorganic thiocyanate to use cannot be given. However, for each specific case the proper amount can be readily determined by those skilled in the art. The examples given herein-after illustrate suitable amounts of the inorganic thiocyanates.

Similarly no definite limits on the amount of the swelling agent that can be used can be given. The amount to be used will vary, for example, depending on the factors named in connection with the inorganic thiocyanates. However, the proper amount to use in a given case can be readily determined by those skilled in the art and is illustrated by the examples given hereinafter.

The present invention or discovery fills a definite need in the printing art. By means of it organic derivative of cellulose (especially cellulose acetate) textile fabrics, colored with dischargeable dyes, can be successfully discharge printed commercially. Again "color on color discharge printing" of cellulose acetate textile fabrics, so far as we are aware, is made commercially possible for the first time. Also in the case of "discharged dyed style" printing clearer and sharper defined patterns are obtained. Likewise, where screen printing is employed the use of our invention or discovery also permits considerably more pieces of goods to be printed before the screen is rendered unsuitable for use.

The following examples illustrate the invention or discovery:

#### EXAMPLE 1

A fabric composed approximately of 50% cellulose acetate and 50% viscose rayon by weight was dyed by the single bath method in the customary manner with  $\frac{3}{4}$  % of 2,4-dinitro-6-monoethylsulfoneamidobenzeneazo - (1,6') - 1' -  $\beta$ , $\gamma$  - dihydroxypropyl-7'-methyl-1,2,3,4 - tetrahydroquinoline having the formula:



(based on the weight of the acetate content) and 1 1/8 % of a commercial preparation of Colour Index Dye 406 (based on the weight of the viscose rayon) dried and impregnated with a solution of the following proportions:

Ounces  
Zinc thiocyanate solution (sp. gr. 1.30) containing 44% zinc thiocyanate by weight 6  
Thiodiglycol 2  
Water 112

The textile fabric was then passed straight through the nip of a two-roll padding machine

with the pressure on the squeeze rollers adjusted so as to allow the textile fabric to retain about 96% of its weight of the above solution. The textile fabric was then carefully dried in a net drier and then printed on a roller printing machine with the discharge pastes made up in the proportions indicated hereinafter. The discharge pastes are applied by separate rollers, the "White Discharge Paste" being applied first.

#### White discharge paste

|                                                           | Ounces |
|-----------------------------------------------------------|--------|
| Textile gum, solubilized Gum Karaya containing 20% solids | 5      |
| Sodium formaldehyde-sulfoxylate 100%                      | 3      |
| Thiodiglycol                                              | 1.6    |
| Water                                                     | 3      |

#### Vat color discharge paste

|                                                | Ounces |
|------------------------------------------------|--------|
| Colour Index Dye 1217 (commercial preparation) | 20     |
| Vat gum paste                                  | 108    |

#### Vat gum paste

|                                      | Ounces      |
|--------------------------------------|-------------|
| British gum                          | ounces 38.4 |
| Modified starch                      | do 14.4     |
| Potassium carbonate (96-98%)         | do 6        |
| Sodium carbonate (58% Na2O)          | do 6        |
| Sodium formaldehyde-sulfoxylate 100% | do 20       |
| Triethylene glycol                   | do 9        |
| Anthraquinone paste (30%)            | do 2.25     |
| Water                                | pounds 6.5  |
| Dry caustic soda                     | ounces 2    |

After printing the textile fabric was dried in the usual manner and then padded on a regular printing machine with a milled stippled roller with a solution containing 3 oz. of 100 volume hydrogen peroxide per gallon of 4% gum tragacanth paste (this mixture was freshly made up). The padding solution was applied only to the face of the printed material in the usual manner and the adjustment of the engraving and set of the machine were made so as to allow not over a 12.5% pick-up on the weight of the textile fabric. The material was then carefully dried in the usual manner and aged in a vat ager for a period of 6 to 8 minutes. The printed and aged textile fabric was then developed in the usual manner for vat colors and then dried. A sharp white and orange discharge was obtained on a bright blue ground.

#### EXAMPLE 2

A fabric composed approximately of 50% cellulose acetate and 50% cotton by weight is treated in accordance with the procedure described in Example 1. A sharp white and orange discharge was similarly obtained on a bright blue ground.

#### EXAMPLE 3

A fabric composed approximately of 50% cellulose and 50% cuprammonium silk by weight was treated in accordance with the procedure described in Example 1. A sharp white and orange discharge was likewise obtained on a bright blue ground.

A fabric composed of 50% by weight of cellulose acetate and 50% by weight of regenerated cellulose can similarly be treated in accordance with the procedure described in Example 1 to obtain a sharp white and orange discharge on a

The textile fabric was then passed straight through the nip of a two-roll padding machine

bright blue ground. Cellulose acetate propionate or cellulose acetate butyrate, for example, can be substituted for the cellulose acetate of the fabrics of Example 1, 2 and 3 and the procedure described in Example 1 carried out to obtain sharp white and orange discharges on a bright blue ground. It will be understood, of course, that cellulose acetate propionate or cellulose acetate butyrate, for example, can also be substituted for cellulose acetate in the examples which follow.

## EXAMPLE 4

A fabric containing approximately 50% by weight of cellulose acetate and 50% by weight viscose rayon is dyed a tomato red shade with  $\frac{1}{4}\%$  of 4-nitrobenzeneazo(1,1')-2'-methyl-4'-di- $\beta$ -hydroxyethylaminobenzene having the formula:



and  $\frac{1}{48}\%$  of 2-methoxy-5-chlorobenzeneazo(1,2')-5'-monomethyl-1',3'-cyclohexadione having the formula:



based on the weight of the cellulose acetate content, and  $\frac{1}{2}\%$  of a commercial preparation of Prototype Dye 79,  $\frac{1}{64}\%$  a commercial preparation of Prototype Dye 24 and  $\frac{1}{32}\%$  of a commercial preparation of Prototype Dye 19 based on the weight of the viscose rayon content. The textile fabric was dyed directly by the usual single bath method, dried and then impregnated with a solution having the following proportions:

|                                                                                               | Ounces |
|-----------------------------------------------------------------------------------------------|--------|
| Aluminum thiocyanate solution containing 28% of aluminum thiocyanate by weight (sp. gr. 1.18) | 6.98   |
| Thiodiglycol                                                                                  | 2      |
| Water                                                                                         | 112    |

The textile fabric was passed straight through the nip of a two-roller padding machine with the pressure on the squeeze rollers adjusted so as to allow the padded textile fabric to retain about 90% of its weight of the above solution. It was then carefully dried in a net drier and then printed by the hand-block-screen method of printing with a paste having the following composition:

|                                                           | Ounces |
|-----------------------------------------------------------|--------|
| Sodium formaldehyde-sulfoxylate 100%                      | 3      |
| Thiodiglycol                                              | 1.5    |
| Water                                                     | 6      |
| Textile gum, solubilized Gum Karaya containing 20% solids | 10     |

After printing the textile fabric with the printing paste just described, the textile fabric was dried in the usual manner, then aged for 8-10 minutes in a chimney ager at 101-106° C., rinsed and dried. White objects which are very sharp in detail are obtained on a red ground.

The above procedure was carried out without

impregnating the dyed textile fabric with an inorganic thiocyanate solution and the resulting printed fabric had a very noticeable halo around the edges and the pattern was considerably "flushed."

## EXAMPLE 5

Fabrics containing approximately 50% by weight of cellulose acetate and 50% by weight cotton; 50% by weight of cellulose acetate and 50% by weight cuprammonium silk can be substituted for the fabric of Example 4 and the procedure of Example 4 carried out to obtain white objects which are very sharp in detail on a red ground in each instance.

## EXAMPLE 6

A satin textile fabric composed wholly of cellulose acetate was dyed a light brown color employing the single bath method in the customary manner with a mixture (by weight on the fabric) of 0.5% of 4-nitrobenzeneazo (1,1')-3'-chloro-4'-mono- $\beta$ -hydroxyethylaminobenzene, 0.5% of 2,4-dinitro-6-monoethylsulfone-amidebenzenearzo (1,6')-1'- $\beta$ , $\gamma$ -dihydroxypropyl-7'-methyl-1,2,3,4-tetrahydroquinoline and 0.25% of 4-nitrobenzeneazo(1,1')-2'-methyl-4'-di- $\beta$ -hydroxyethylaminobenzene. Following the dyeing operation, the textile fabric was dried and then treated with a solution made up in the following proportions:

|                                                                                    |            |
|------------------------------------------------------------------------------------|------------|
| Zinc thiocyanate solution containing 44% zinc thiocyanate by weight (sp. gr. 1.30) | ounces 6   |
| Triethylene glycol                                                                 | do 4       |
| Water                                                                              | quarts 3.5 |

The textile fabric was passed straight through the nip of a two-roll padding machine with the pressure on the squeeze rollers adjusted so as to allow the padded textile fabric to retain about 95% of its weight of the above solution. It was then carefully dried in a net drier and then printed by the hand-block-screen method of printing with a paste made up in the following proportions:

|                                                          | Ounces |
|----------------------------------------------------------|--------|
| Sodium formaldehyde sulfoxylate 100%                     | 3      |
| Thiodiglycol                                             | 1.5    |
| Water                                                    | 6      |
| Textile gum solubilized Gum Karaya containing 20% solids | 10     |

After printing the textile fabric with the printing paste just described the textile fabric was dried in the usual manner, then aged for 8-10 minutes in a chimney ager at 101-106° C., rinsed and dried. A white object which was very sharp in detail was obtained on a light brown ground.

The textile fabric of the example dyed as described above can also be subjected to a roll printing operation in accordance with the procedure described in Example 1, except that the zinc thiocyanate mixture described above is employed instead of that of the example. A white and orange discharge on a brown ground is obtained.

## EXAMPLE 7

A taffeta textile fabric composed wholly of cellulose acetate was dyed a light brown color employing the dye mixture of Example 6. Following the dyeing operation, the textile fabric

was dried and then treated with a solution made up in the following proportions:

Zinc thiocyanate solution containing 44% zinc thiocyanate by weight (sp. gr. 1.30)

ounces 6 15

$\text{CH}_3\text{CNCH}_2\text{CH}_2\text{OCCH}_3$ , do 4

Water quarts 3.5

The textile fabric was then passed straight through the nip of a two-roll padding machine with the pressure on the squeeze rollers adjusted so as to allow the textile fabric to retain about 96% of its weight of the above solution. The textile fabric was then carefully dried in a net drier and simultaneously printed on a roller printing machine with the discharge paste made up in the proportions indicated hereinafter.

*White discharge paste*

|                                                          | Ounces |
|----------------------------------------------------------|--------|
| Textile gum solubilized Gum Karaya containing 20% solids | 5      |
| Sodium formaldehyde sulfoxylate 100%                     | 3      |
| Thiodiglycol                                             | 1.6    |
| Water                                                    | 3      |

After printing, the textile fabric was dried in the usual manner and then padded on a regular printing machine with a milled stippled roller with a solution containing 3 oz. of 100 volume hydrogen peroxide per gallon of 4% gum tragacanth paste (this mixture was freshly made up). The padding solution was applied only to the face of the printed material in the usual manner and the adjustment of the engraving and set of the machine were made so as to allow not over a 12.5% pick-up on the weight of the textile fabric. The material was then carefully dried in the usual manner and aged in a vat ager for a period of 6 to 8 minutes. The printed and aged textile fabric was then developed in the usual manner for vat colors and then dried. A white discharge was obtained on a light brown ground.

The colored cellulose acetate textile fabric of the example can also be screen printed in accordance with the procedure described in Example 6 to obtain white objects which are sharp in detail on a light brown ground.

**EXAMPLE 8**

A textile fabric containing approximately 50% by weight of cellulose acetate propionate and 50% by weight viscose rayon was treated exactly in accordance with the procedure described in Example 2. A white object which was very sharp in detail was obtained on a red ground.

A textile fabric containing approximately 50% by weight of cellulose acetate propionate and 50% by weight cotton and a textile fabric containing approximately 50% by weight of cellulose acetate propionate and 50% by weight cuprammonium silk can be substituted for the textile fabric of the example and subjected to the identical procedure to obtain prints substantially the same as that of the example.

It will be understood that the foregoing examples are intended to be illustrative and not limitative of our invention. Thus, as has been indicated hereinbefore, other inorganic thiocyanates can be used in place of the zinc thiocyanate and aluminum thiocyanate employed in the examples. The following tabulation sets forth suitable amounts of various inorganic thiocyanates which

can be used to treat the colored textile fabrics indicated herein in accordance with the process of our invention or discovery.

| Inorganic thiocyanate | Spr. Gr. | Oz.  | Percent Inorganic Thiocyanate By Weight |
|-----------------------|----------|------|-----------------------------------------|
| Manganous thiocyanate | (solid)  | 4.68 | 66                                      |
| Barium thiocyanate    | (solid)  | 3.78 | 81                                      |
| Magnesium thiocyanate | 1.28     | 6.18 | 41                                      |
| Calcium thiocyanate   | 1.22     | 6.60 | 34                                      |
| Sodium thiocyanate    | solid    | 1.22 | C. P.                                   |
| Potassium thiocyanate | solid    | 1.46 | C. P.                                   |

Any of the above thiocyanates can be added to 112 oz. of water and 2 oz. of thiodiglycol to form suitable mixtures for treating the colored textile fabric prior to the discharge printing operation. The inorganic thiocyanate padding solution or mixture can be made up to contain only the inorganic thiocyanate compound as indicated above but generally a swelling agent is included. Suitable amounts of the swelling agent to be incorporated into the padding solution have been indicated in the examples. It will be clearly understood that the thiocyanates tabulated above can be substituted for the thiocyanates of the examples to obtain the same or substantially equivalent results. Also it is to be clearly understood that the process of our invention or discovery is not limited to the use of the particular swelling agents disclosed in the examples as generally similar amounts of the other swelling agents indicated herein can be employed.

Other inorganic thiocyanate solutions that can be employed for treating or padding the colored textile fabric prior to the discharge printing operation are listed hereinafter.

**EXAMPLE A**

|                                              | Ounces |
|----------------------------------------------|--------|
| Aluminum thiocyanate solution (sp. gr. 1.30) | 7      |
| Water                                        | 112    |

**EXAMPLE B**

|                                               | Ounces |
|-----------------------------------------------|--------|
| Magnesium thiocyanate solution (sp. gr. 1.28) | 6      |
| Water                                         | 112    |

**EXAMPLE C**

|                                             | Ounces |
|---------------------------------------------|--------|
| Calcium thiocyanate solution (sp. gr. 1.22) | 7      |
| Sulfated fatty alcohol                      | 0.1    |
| Water                                       | 112    |

**EXAMPLE D**

|                       | Ounces |
|-----------------------|--------|
| Manganous thiocyanate | 5      |
| Triethyleneglycol     | 5      |
| Salicylic acid        | 1      |
| Water                 | 112    |

**EXAMPLE E**

|                                               | Ounces |
|-----------------------------------------------|--------|
| Magnesium thiocyanate solution (sp. gr. 1.28) | 6      |
| Citric acid                                   | 3      |
| Water                                         | 112    |

**EXAMPLE F**

|                                               | Ounces |
|-----------------------------------------------|--------|
| Aluminum thiocyanate solution (sp. gr. 1.30)  | 4      |
| Magnesium thiocyanate solution (sp. gr. 1.28) | 3      |
| Water                                         | 112    |

The amounts of the inorganic thiocyanates and swelling agents indicated above are not critical as greater or lesser amounts can be employed. In the claims the expression "a substantial amount" has been used with reference to the amount of the inorganic thiocyanate or swelling agent incorporated into the colored textile fabric. This expression means only that "an effective amount," that is, an amount sufficient to exert a perceptible beneficial effect is employed—as compared to the result obtained without the use of either an inorganic thiocyanate or a swelling agent. Beneficial amounts of the inorganic thiocyanates and swelling agents to use have been taught hereinbefore.

The inorganic thiocyanates can be used alone or in combination with each other. Thus, zinc thiocyanate can be used alone or in conjunction with either calcium thiocyanate or magnesium thiocyanate or with both these thiocyanates, for example. As the combinations which can be employed are obvious additional combinations have been omitted as unnecessary. Similarly, one or more swelling agents can be employed in conjunction with the inorganic thiocyanates. To illustrate, thiodiglycol and triethylene glycol, triethylene glycol and diethylene glycol or thiodiglycol, glycerol and tetraethyleneglycol can be employed. Other combinations that can be employed are readily apparent.

As will be apparent to those skilled in the art to which this invention or discovery is directed and as indicated hereinbefore, any dischargeable dye for the colored textile fabric can be employed in the process of the invention or discovery. Additional dyes whose dyeings can be discharged from cellulose acetate include, for example, 4-nitrobenzeneazo (1,1')-4'-N-ethyl-4'-N- $\beta$ -hydroxyethylaminobenzene (Prototype Dye 244), 2,4-dinitrobenzeneazo (1,1')-2'-methyl-5'-methoxy-4'-N- $\beta$ , $\gamma$ -dihydroxypropylaminobenzene, Prototype Dye 236 (4-nitrobenzeneazo (1,1')-2'-methyl-4'-N,N-di- $\beta$ -hydroxyethylaminobenzene), Prototype Dye 238 (2-chloro-4-nitrobenzeneazo (1,1')-2-methyl-4'-N,N-di- $\beta$ -hydroxyethylaminobenzene) and Prototype Dye 242 (4-acetylaminobenzeneazo (1,1')-2'-hydroxy-5'-methylbenzene). Similarly, many other dyes in addition to those specifically indicated can be used in the "color on color" discharging operation. To illustrate, Colour Index Dye 1217, Prototype Dye 107, Flavanthrone, Colour Index Dye 1151, Colour Index Dye 1101 and Colour Index Dye 1104 can be employed. The dyes listed herein are merely illustrative as other dyes are known to those skilled in the art that can be employed. Finally, dyes (such as Prototype Dye 20, for example) other than those specifically disclosed can be used to produce dischargeable dyeings on viscose, cotton and cuprammonium silk, for example. The particular dye or dyes employed constitute little or no part of the invention as any suitable known dyes or any suitable dyes developed in the future can be employed. Colour Index or prototype numbers given are those given in the "1941 Year Book of the American Association of Textile Chemists and Colorists." In a few cases the prototype number does not appear in the book just referred to and in those cases, the number appears, for example, in the "1941 Year Book of the American Association of Textile Chemists and Colorists, Vol. XXI."

The discharge-printing pastes disclosed are intended to be illustrative and not limitative since,

within the teachings of the invention, considerable variation can be made in these printing pastes as is well known to those skilled in the art. The printing pastes disclosed, however, have been found to be quite satisfactory.

The term "dry" as used in the claims is not intended to mean that the textile fabric must be entirely moisture-free. All that is required is that the fabric be "relatively" or "substantially" dry. That is the fabric need be just dry enough that the printing operation or operations can be satisfactorily carried out. Normally the fabric is quite dry. The amount of drying required for satisfactory operation in any given case can be readily determined.

While our invention or discovery has been described more particularly in connection with the discharge printing of cellulose acetate—the most important member of the organic derivative of cellulose class—it is applicable to the discharge printing of other organic derivatives of cellulose such as those named hereinbefore. Again, while all regenerated celluloses have not been tested, it would appear that this general class of substances illustrated by viscose and cuprammonium silk, for example, can be present in the textile fabric.

The single bath method of dyeing referred to in the examples is well known to those skilled in the art to which this invention or discovery is directed. One satisfactory way of carrying out this method of dyeing is to prepare a paste from an intimate admixture of the dye or dyes to be employed with a dispersing or solubilizing agent and to add this paste to the dyebath. The dye paste can be prepared from water and the mixture of dye and dispersing agent. We have found that a dyebath containing 25 parts by weight of water to 1 part by weight of cloth is very satisfactory. Preferably a small amount of a wetting agent is also present in the dyebath during the dyeing operation. 1% of 1% (by weight on the cloth) of sodium lauryl sulfate has been found satisfactory for this purpose. The dyeing operation is completed by subjecting the cloth to treatment in the dyebath at a temperature of 190° F. for 2½ hours. It is to be clearly understood, however, that the single dye bath method of dyeing just described is illustrative and not limitative as many variations are possible.

We claim:

1. The process of discharge printing a colored organic derivative of cellulose textile fabric which comprises treating the colored textile fabric with an acid inorganic thiocyanate whereby a substantial amount of the acid inorganic thiocyanate is impregnated in the fabric, passing the textile fabric in dried condition to a roller printing machine and discharge printing the colored textile fabric containing the thiocyanate with an alkali metal formaldehyde-sulfoxylate white discharge printing paste and an alkali metal formaldehyde-sulfoxylate vat color discharge printing paste whereby white and colored objects, wherein the color of the colored objects differs from that of the colored textile fabric, are obtained on the colored textile fabric.

2. The process of discharge printing a colored organic derivative of cellulose textile fabric which comprises treating the colored textile fabric with a solution of an acid inorganic thiocyanate and thiodiglycol, whereby a substantial amount of the acid inorganic thiocyanate and thiodiglycol is impregnated in the textile fabric, drying the textile fabric, passing the dried textile fabric to

a roller printing machine and discharge printing the colored textile fabric containing the thiocyanate with an alkali metal formaldehyde-sulfoxylate white discharge printing paste and an alkali metal formaldehyde-sulfoxylate vat color discharge printing paste whereby white and colored objects, wherein the color of the colored objects differs from that of the colored textile fabric, are obtained on the colored textile fabric.

3. The process of discharge printing a colored cellulose acetate textile fabric which comprises treating the colored textile fabric with an acid inorganic thiocyanate whereby a substantial amount of the acid inorganic thiocyanate is impregnated in the fabric, passing the textile fabric in dried condition to a roller printing machine and discharge printing the colored textile fabric containing the thiocyanate with an alkali metal formaldehyde-sulfoxylate white discharge printing paste and an alkali metal formaldehyde-sulfoxylate vat color discharge printing paste whereby white and colored objects, wherein the color of the colored objects differs from that of the colored textile fabric, are obtained on the colored textile fabric.

4. The process of discharge printing a colored cellulose acetate textile fabric which comprises treating the colored textile fabric with a solution of an acid inorganic thiocyanate and thiodiglycol, whereby a substantial amount of the acid inorganic thiocyanate and thiodiglycol are impregnated in the textile fabric, drying the textile fabric and passing the dried textile fabric to a roller printing machine and discharge printing the colored textile fabric containing the thiocyanate with an alkali metal formaldehyde-sulfoxylate white discharge printing paste and an alkali metal formaldehyde-sulfoxylate vat color discharge printing paste whereby white and colored objects, wherein the color of the colored objects differs from that of the colored textile fabric, are obtained on the colored textile fabric.

5. The process of discharge printing a colored organic derivative of cellulose textile fabric which comprises treating the colored textile fabric with an acid inorganic thiocyanate and an organic swelling agent for the textile fabric, whereby a substantial amount of the acid inorganic thiocyanate and the organic swelling agent is impregnated in the fabric, passing the textile fabric in dried condition to a roller printing machine and discharge printing the colored textile fabric containing the thiocyanate and the organic swelling agent with an alkali metal formaldehyde-sulfoxylate white discharge printing paste and an alkali metal formaldehyde-sulfoxylate vat color discharge printing paste, whereby white and colored objects, wherein the color of the colored objects differs from that of the colored textile fabric, are obtained on the colored textile fabric.

6. The process of discharge printing a colored organic derivative of cellulose textile fabric which comprises treating the colored textile fabric with a solution of an acid inorganic thiocyanate and an organic polyhydric-alcohol swelling agent, whereby a substantial amount of the acid inorganic thiocyanate and the organic polyhydric-alcohol swelling agent is impregnated in the fabric, drying the textile fabric and passing the dried textile fabric to a roller printing machine and discharge printing the colored textile fabric containing the thiocyanate and the swelling agent

with an alkali metal formaldehyde-sulfoxylate white discharge printing paste and an alkali metal formaldehyde-sulfoxylate vat color discharge printing paste, whereby white and colored objects, wherein the color of the colored objects differs from that of the colored textile fabric, are obtained on the colored textile fabric.

7. The process of discharge printing a colored cellulose acetate textile fabric which comprises treating the colored textile fabric with an acid inorganic thiocyanate and an organic swelling agent for the textile fabric, whereby a substantial amount of the acid inorganic thiocyanate and the organic swelling agent is impregnated in the fabric, passing the textile fabric in dried condition to a roller printing machine and discharge printing the colored textile fabric containing the thiocyanate and the organic swelling agent with an alkali metal formaldehyde-sulfoxylate white discharge printing paste and an alkali metal formaldehyde-sulfoxylate vat color discharge printing paste, whereby white and colored objects, wherein the color of the colored objects differs from that of the colored textile fabric, are obtained on the colored textile fabric.

8. The process of discharge printing a colored cellulose acetate textile fabric which comprises treating the colored textile fabric with a solution of an acid inorganic thiocyanate and an organic polyhydric-alcohol swelling agent, whereby a substantial amount of the acid inorganic thiocyanate and the organic polyhydric-alcohol swelling agent is impregnated in the fabric, drying the textile fabric and passing the dried textile fabric to a roller printing machine and discharge printing the colored textile fabric containing the thiocyanate and the swelling agent with an alkali metal formaldehyde-sulfoxylate white discharge printing paste and an alkali metal formaldehyde-sulfoxylate vat color discharge printing paste, whereby white and colored objects, wherein the color of the colored objects differs from that of the colored textile fabric, are obtained on the colored textile fabric.

HERBERT G. SCULL.  
JAMES G. McNALLY.

#### REFERENCES CITED

The following references are of record in the file of this patent:

#### UNITED STATES PATENTS

| Number    | Name    | Date          |
|-----------|---------|---------------|
| 1,398,357 | Briggs  | Nov. 29, 1921 |
| 1,651,639 | Smith   | Dec. 6, 1927  |
| 1,874,176 | Ellis   | Aug. 30, 1932 |
| 1,898,211 | Fenche  | Feb. 21, 1933 |
| 1,912,008 | Powers  | May 30, 1933  |
| 1,931,108 | Downing | Oct. 17, 1933 |
| 1,957,491 | Dreyfus | May 8, 1934   |
| 1,963,121 | Ellis   | June 19, 1934 |
| 1,972,137 | Ellis   | Sept. 4, 1934 |
| 1,981,907 | Downing | Nov. 27, 1934 |
| 2,031,594 | Dreyfus | Feb. 25, 1936 |
| 2,037,013 | Dreyfus | Apr. 14, 1936 |
| 2,065,125 | Dreyfus | Dec. 22, 1936 |
| 2,289,461 | Salvin  | July 14, 1942 |

#### FOREIGN PATENTS

| Number  | Country       | Date          |
|---------|---------------|---------------|
| 285,942 | Great Britain | Feb. 23, 1928 |

**Certificate of Correction**

Patent No. 2,436,059.

February 17, 1948.

**HERBERT G. SCULL ET AL.**

It is hereby certified that errors appear in the printed specification of the above numbered patent requiring correction as follows: Column 4, line 30, for the word "out" read *our*; line 41, for the word "indicated" read *intended*; column 7, line 4, for "Example" read *Examples*; column 11, line 71, for "1941" read *1944*; and that the said Letters Patent should be read with these corrections therein that the same may conform to the record of the case in the Patent Office.

Signed and sealed this 27th day of April, A. D. 1948.

[~~initials~~]

**THOMAS F. MURPHY,**  
*Assistant Commissioner of Patents.*